# EUROPEAN PATENT SPECIFICATION

(11) **EP 3 250 539 B1**
(45) Date of publication and mention of the grant of the patent: **17.04.2024**
(21) Application number: 16702765.5
(22) Date of filing: 26.01.2016
(51) Int. Cl.: C06B 27/00, C06B 33/00, C06B 43/00

(54) **REACTIVE MATERIALS**
REAKTIVE MATERIALIEN
MATÉRIAUX RÉACTIFS

(30) Priority: 27.01.2015 GB 201501336
(43) Date of publication of application: 06.12.2017
(73) Proprietor: BAE Systems PLC, London SW1Y 5AD (GB)
(72) Inventor: FLYNN, Dennis, Joseph, Usk Monmouthshire NP15 1XL (GB); KENNETT, Eric, John, Washington Tyne and Wear NE37 1PA (GB)
(74) Representative: BAE SYSTEMS plc Group IP Department
(86) International application number: PCT/GB2016/050161
(87) International publication number: WO 2016/120605

(56) References cited:
- EP-A1- 0 051 324
- EP-A1- 1 286 129
- EP-A2- 1 348 683
- WO-A2-2007/086830
- US-A- 3 956 038
- US-A- 4 131 498
- US-A- 4 381 692
- US-A1- 2003 070 540
- US-A1- 2005 199 323

## Description

The invention relates to high density reactive materials, preferably materials with a high density and exothermic output.

High Density reactive materials (HDRM) are a new emerging class of materials http://en.wikipedia.org/wiki/Reactive_materials, which have higher densities than conventional reactive materials such that they may provide enhanced performance with mechanical properties suitable for application in a broad range of weapon systems. This includes potential for effective transfer of Kinetic Energy in impact penetrators, fragments and other systems, whilst offering an additional advantage of providing a further exothermic output under explosive loading or following High Velocity impact.

US2003/0070540 is directed to a projectile shell having a core region which contains a reactive composition comprised of a reactive metal and an oxidizer.
US 4 381 692 A discloses high-density reactive material for use in a munition.
US 2005/199323 A1 discloses high-density reactive material comprising hafnium. EP 0 051 324 A1 is directed to metallic fuel/incendiary compositions.
US 4 131 498 A is directed to incendiary compositions Zr or Hf with a binder. EP 1 348 683 A2 is directed to extrudable high density reactive materials based on metal and metal oxides. EP 1 286 129 A1 is directed to an incendiary composition comprising titanium sponge in an epoxide resin or a polyester resin.
WO 2007/086830 is directed to nano powders, particularly metal and metal oxides. US 3 956 038 A is directed to pyrotechnic compositions in a polymer binder

According to a first aspect of the invention there is provided a high density reactive material composition comprising,
A) at least two separate group 4 metals, present in the range of from 40 to 90%wt, wherein at least one of the group 4 metals is hafnium, wherein hafnium is present in the range of from 15% to 51 %..
B) at least one alloying element, selected from boron or carbon present in the range of from 5 to 55%wt
C) wherein the at least two group 4 metals are encapsulated by a fluoroelastomer binder present in the range of 1-10%wt.
wherein said reagents A), B), C) and optional pressing aids are present in substantially 100%wt.

The reagent B) is selected from alloying elements carbon or boron. The boron may be present in an amount 5 to 20%wt, preferably 10%wt.

The reagent A) group 4 metals are group 4, d-block (transition metals) such as titanium, zirconium, and hafnium. These metals offer high densities, and the specific selection of two different group 4 options offers a chance to target specific density ranges for the final composition whilst retaining similar reactivity.

At least one of the group 4 metals is hafnium. Preferably the hafnium is present in the range of from 15 to 30%wt. The specific inclusion of Hafnium, in the range of from 15 to 30%wt, or more preferably in the range of 20 to 25%wt,which provides a significant increase to the overall effective density of the consolidated composition, for a relatively minor volumetric inclusion.

The group 4 metals may offer a range of morphologies - comprising nano, sub micron, or micron sized particulates. The at least two group 4 metals may be selected to maximise mixing capability to promote uniformity of distribution (these may be substantially the same size, or targeted different size ranges to achieve a specific multimodal distribution, such as a bimodal distribution.

The reagent B may be selected from nano, sub micron, or micron sized particulates, such that upon intimate mixing with group 4 metals, may support/provide a homogenous mixture. The particulate size of the group 4 metals and reagent B materials may be selected to provide multimodal distributions.

The reagent C) binder is at least one fluoroelastomer binder. The fluoroelastomer binder may be selected from a range of materials such as for example hexafluoropropylene, vinylidene fluoride, terpolymers of tetrafluoroethylene, vinylidene fluoride and hexafluoropropylene (HFP), perfluoromethylvinylether, THV 220, and PTFE, preferably a Viton, more preferably Viton A.

The reagent C) binder may preferably be present in the in the range of from 3 to 7%wt, preferably 5%wt.

According to a further aspect of the invention there is provided a munition comprising a portion of the consolidated composition as defined herein. The portion of the munition may comprise all, substantially all or part of a munition. The munition may such as for example be a direct fire or indirect fire munition. The munition may be kinetic energy or chemical energy munition or a combination thereof, such as, for example a projectile, shell, casing, shaped charge liner, preformed fragments or mortar.

The munition may be a kinetic energy projectile such as for example, such as a round, from a small calibre ordnance, a medium calibre projectile such as, for example calibres of 30- 40mm and above, penetrator rods or flechettes. The projectile may comprise or contain only a monolithic projectile of consolidated composition as defined herein. Certain medium calibre projectiles typically comprise a high explosive, the use of a projectile (small or medium calibre) comprising or containing only a consolidated composition according to the invention may provide an insensitive munition.

The munition may be a gun launched shell, such as for example, 105mm or 155mm, wherein part, substantially all or all of the shell casing is a composition as defined herein. The composition may be prepared to form pre formed fragments which are further consolidated to form a shell casing. In a munition subjected to a high set back force, such as a gun launched munition, preferably there is a higher percentage weight of fluoroelastomer binder.

The munition may comprise at least one layer deposed thereon of the composition as defined herein.

The casing of the munition may be subjected to prompt break up, ignition and burn to enhance blast effectiveness.

The particulates of the composition may not be consolidated and may be available as agglomerates/clumps, and may be ignited as such, and undergo ignition and continue to burn in flight. This may offer enhancement to blast and after burn or Kinetic Energy transfer to targets at range.

The composition either solid or agglomerates may be ejected, or projected , in such a manner to retain physical form/mass and associated Kinetic Energy allowing reaction on impact with targets at a specific thresh-hold impact velocity causing shock reaction and ignition of the material on the surface or within the target structure.

According to a further aspect not according to the invention there is provided a method of preparing a high density reactive material as defined herein, such as for example, dead load pressing, isostatic pressing, hot sintering, to provide a composition which may be consolidated to form a structural casing or projectile.

**Table 1 # compounds no longer form part of the invention**

| | Ingredient 1 | | Ingredient 2 | | Ingredient 3 | | Ingredient 4 | | Overall |
|---|---|---|---|---|---|---|---|---|---|
| Ref | Name | Wt % | Name | Wt % | Name | Wt % | Name | Wt % | Effective Density by Wt fraction |
| #1a | Zirconium | 25% | CuO | 50% | Viton A | 5% | Hafnium | 20% | 6.27 |
| 21a | Titanium | 35% | Boron | 10% | Viton A | 5% | Hafnium | 50% | 5.46 |
| 23a | Hafnium | 51% | Boron | 10% | Viton A | 5% | Zirconium | 34% | 6.28 |
| #25a | Titanium | 25% | CuO | 45% | Viton A | 5% | Hafnium | 25% | 5.79 |
| #26a | Hafnium | 20% | CuO | 45% | Viton A | 5% | Zirconium | 30% | 6.28 |
| #28a | Zirconium | 45% | THV220 | 10% | | | Tungsten | 45% | 5.71 |
| #29a | Hafnium | 79% | THV220 | 10% | | | Zirconium | 11% | 6.29 |
| #U1 | Zirconium | 45% | Zinc | 40% | | | Tungsten | 15% | 7.53 |

Table 1 provides a number of examples where the composition comprises a group 4 metal present in the range of from 45 to 95%wt. the materials are sintered, preferably using both elevated temperatures and pressure with the a binder and optional pressing aids to facilitate consolidation.

**Table 2 # compounds no longer form part of the invention**

| | Reagent A | | Reagent B | | Reagent C | | Reagent A | | Overall |
|---|---|---|---|---|---|---|---|---|---|
| Ref | Name | Wt % | Name | Wt % | Name | Wt % | Name | Wt % | Effective Density by Wt fraction |
| #1a | Zirconium | 25% | CuO | 50% | Viton A | 5% | Hafnium | 20% | 6.27 |
| 21a | Titanum | 35% | Boron | 10% | Viton A | 5% | Hafnium | 50% | 5.46 |
| 23a | Hafnium | 51% | Boron | 10% | Viton A | 5% | Zirconium | 34% | 6.28 |
| #25a | Titanium | 25% | CuO | 45% | Viton A | 5% | Hafnium | 25% | 5.79 |
| #26a | Hafnium | 20% | CuO | 45% | Viton A | 5% | Zirconium | 30% | 6.28 |

Table 2 above, provides preferred examples of compositions, wherein at least two different group 4 metals are selected.

The group 4 metals may be encapsulated or a passivation layer, or sacrificial layer to prevent reaction with air, moisture or unwanted reactions with the other reagents, until activated in the designed mode of use. The group 4 metals may be encapsulated with at least one inert material, to prevent reaction with moisture or air. The group 4 metal is premixed with reagent C) a fluoroelastomer binder. The coating/microencapsulation of the group 4 metal may prevent combustion in air during the sintering process.

## Claims

1. A high density reactive material composition comprising,
A) at least two separate group 4 metals, present in the range of from 40 to 90%wt, wherein at least one of the group 4 metals is hafnium, wherein hafnium is present in the range of from 15% to 51 %..
B) at least one alloying element, selected from boron or carbon present in the range of from 5 to 55%wt
C) wherein the at least two group 4 metals are encapsulated by a fluoroelastomer binder, present in the range of 1-10%wt.
wherein said reagents and optional pressing aids are present in substantially 100%wt.

2. A composition according to claim 1, wherein the hafnium is present in the range of from 15 to 30%wt

3. A composition according to claim 1 or 2, wherein said fluoroelastomer binder is present in the in the range of from 3 to 7%wt.

4. A high density reactive material composition according to any one of the preceding claims, wherein said consolidated composition comprises an effective density by weight fraction of greater than 5.40.

5. A munition comprising a portion of the consolidated composition according to any one of the preceding claims.

6. A munition according to claim 5, wherein the portion comprises all, substantially all or part of a projectile, shell, casing, shaped charge liner, natural, forced or preformed fragments or a mortar.

## Patentansprüche

1. Zusammensetzung eines reaktiven Materials hoher Dichte, umfassend,
A) mindestens zwei separate Metalle der Gruppe 4, die in dem Bereich von 40 bis 90 Gew.-% vorhanden sind, wobei mindestens eines der Metalle der Gruppe 4 Hafnium ist, wobei Hafnium in dem Bereich von 15 % bis 51 % vorhanden ist.
B) mindestens ein Legierungselement, das ausgewählt ist aus Bor oder Kohlenstoff, das in dem Bereich von 5 bis 55 Gew.-% vorhanden ist.
C) wobei die mindestens zwei Metalle der Gruppe 4 durch ein Fluorelastomerbindemittel eingekapselt sind, das in dem Bereich von 1 bis 10 Gew.-% vorhanden ist
wobei die Reagenzien und optionalen Presshilfsmittel im Wesentlichen in 100 Gew.-% vorhanden sind.

2. Zusammensetzung nach Anspruch 1, wobei das Hafnium in dem Bereich von 15 bis 30 Gew.-% vorhanden ist.

3. Zusammensetzung nach Anspruch 1 oder 2, wobei das Fluorelastomerbindemittel in dem Bereich von 3 bis 7 Gew.-% vorhanden ist.

4. Zusammensetzung eines reaktiven Materials hoher Dichte nach einem der vorstehenden Ansprüche, wobei die verfestigte Zusammensetzung eine wirksame Dichte nach Gewichtsanteil von mehr als 5,40 umfasst.

5. Munition, umfassend einen Abschnitt der verfestigten Zusammensetzung nach einem der vorstehenden Ansprüche.

6. Munition nach Anspruch 5, wobei der Abschnitt alle, im Wesentlichen alle oder einen Teil eines Geschosses, einer Hülle, eines Gehäuses, einer Hohlladungseinlage, natürlicher, erzwungener oder vorgeformter Fragmente oder eines Mörsers umfasst.

## Revendications

1. Composition de matériau réactif à haute densité comprenant,
A) au moins deux métaux de groupe 4 séparés, présents dans la plage allant de 40 à 90 % en poids, dans laquelle au moins l'un des métaux du groupe 4 est du hafnium, dans laquelle l'hafnium est présent dans la plage de 15 % à 51 %.
B) au moins un élément d'alliage, choisi parmi le bore ou le carbone présent dans la plage allant de 5 à 55 % en poids.
C) dans laquelle les au moins deux métaux du groupe 4 sont encapsulés par un liant fluoroélastomère, présent dans la plage de 1 à 10 % en poids.
dans laquelle lesdits réactifs et auxiliaires de pressage facultatifs sont présents dans sensiblement 100 % en poids.

2. Composition selon la revendication 1, dans laquelle le hafnium de carbone est présent dans la plage de 15 à 30 % en poids.

3. Composition selon la revendication 1 ou 2, dans laquelle ledit liant fluoroélastomère est présent dans la plage allant de 3 à 7 % en poids.

4. Composition de matériau réactif à haute densité selon l'une quelconque des revendications précédentes, dans laquelle ladite composition consolidée comprend une masse volumique efficace en fraction pondérale supérieure à 5,40.

5. Munition comprenant une partie de la composition consolidée selon l'une quelconque des revendications précédentes.

6. Munition selon la revendication 5, dans laquelle la partie comprend tous, sensiblement tout ou partie d'un projectile, une coque, un boîtier, un revêtement de charge façonné, des fragments naturels, forcée ou préformés ou un mortier.
